

K. S. GUITERMAN.  
ELECTROLYTIC PROCESS FOR THE EXTRACTION OF COBALT OXIDS.  
APPLICATION FILED AUG. 26, 1915.  
1,195,211.

Patented Aug. 22, 1916.

Fig. 1



Fig. 2



Kenneth S. Guiterman  
Inventor

By his Attorney

Messrs. & Neelin

# UNITED STATES PATENT OFFICE.

KENNETH S. GUITERMAN, OF NEW YORK, N. Y.

## ELECTROLYTIC PROCESS FOR THE EXTRACTION OF COBALT OXIDS.

1,195,211.

Specification of Letters Patent. Patented Aug. 22, 1916.

Application filed August 26, 1915. Serial No. 47,427.

To all whom it may concern:

Be it known that I, KENNETH S. GUITERMAN, a citizen of the United States, and resident of the city of New York, in the county of New York and State of New York, have invented certain new and useful Improvements in Electrolytic Processes for the Extraction of Cobalt Oxids, of which the following is a specification.

10 This invention relates to an electrolytic process for the extraction of cobalt oxids.

Heretofore the common practice in the extraction of cobalt oxid has been to treat the solution containing the cobalt, which 15 usually exists as a sulfate or as a chlorid, with an oxidizing agent such as bleaching powder to convert the sulfate into an oxid or a hydrated oxid. The solutions, however, are usually impure due to the presence 20 of nickel salts, such as nickel sulfate. When the bleaching powder is added to such an impure solution, its action is selective in that it tends to precipitate first an oxid or hydrated oxid of cobalt and then a salt of 25 nickel is thrown down from the solution. As a result of this fractional precipitative action of the bleaching powder, it is obvious that it is impossible to remove all or even the major portion of the cobalt from the solution without at the same time precipitating 30 some of the nickel. In order, therefore, to finally obtain a pure oxid of cobalt it has been necessary to repeat the operation of fractional precipitation until the quantity 35 of nickel which finally remains with the cobalt is of negligible amount. These manifold operations involve many troublesome delays together with the formation of objectionable intermediate by-products carrying 40 varying amounts of cobalt and nickel which must be re-handled during some future treatment.

I am aware that certain electrolytic processes for the extraction of cobalt oxids have 45 been proposed but numerous difficulties have been encountered in the commercial utilization of these processes which have rendered them objectionable if not entirely inoperative.

50 One of the objects of the present invention is to carry on an electrolytic process for the separation of cobalt from nickel with the recovery of the former as an oxid or hydrated oxid, in such a manner as to render it

free from the objectionable features above 55 suggested and at the same time to recover, in one operation, substantially all of the cobalt in an essentially pure condition free from nickel.

A further object is to obtain oxid or 60 hydrated oxid of cobalt in a substantially pure condition at a very low cost and by a process which is continuous and practically automatic.

In the electrolytic process and as a result 65 of the passage of the electric current through the solution or electrolyte which contains not only cobalt and nickel salts but usually a certain amount of soluble chlorids, such as common salt (NaCl), there is liberated 70 at the anode nascent chlorin gas, which has a tendency to rise to the surface and escape into the atmosphere. This chlorin gas is the essential element in the conversion 75 of the soluble cobalt to the oxid or hydrated oxid of cobalt. The action of the chlorin in accomplishing this result may be briefly summarized as follows: 1. Reaction of the chlorin gas with the electrolyte to form a 80 hypochlorite. 2. Reaction of the hypochlorite with the solution of cobalt to form the hydrated oxid of cobalt (a brownish black precipitate) and some free hydrochloric or sulfuric acid.

In view of the fact that hydrated oxid 85 of cobalt is extremely soluble in even weak acids, it is necessary in this process to provide for the neutralization of any free acids formed in the second reaction defined, in order that the precipitation of the cobalt 90 may proceed in an efficient manner. Such neutralization is accomplished through the continuous addition to the electrolyte of a basic neutralizing agent such as sodium carbonate during the progress of the electrolysis. 95

From the above general outline it is obvious that the efficiency of the process will depend upon two factors, namely: *a.* The formation of the maximum amount of hypochlorite possible. *b.* The correct neutralization of the free acids formed through the precipitation of the cobalt oxid. In general it may be stated that the amount of hypochlorite which can be formed in a solution of this character will be directly in proportion to the amount of gaseous chlorin held in the solution. The efficiency of the 100 105

reaction will, therefore, depend upon the retention of the chlorin gas, formed at the anode in the electrolyte, and the prevention of its escape into the atmosphere above the 5 electrolytic cell.

Accordingly another object of the invention is to provide means for giving the solution a directional flow designed to prevent the natural upward flow of the liberated 10 chlorin gas and to retain the same in intimate chemical association with the solution under treatment. Another reason for retaining this gaseous chlorin is that its release would also be highly objectionable 15 owing to its injurious effect upon the lungs of workmen in the vicinity. I attain this latter object broadly by causing the electrolytic solution to pass across the electrodes in a continuous stream, in a direction and at a 20 speed sufficient to retain the chlorin gas in the solution. Preferably the solution is fed in at the top of an electrolytic vat and the precipitates withdrawn from the bottom of the vat in a continuous stream.

25 By means of my process also, the hydrated oxid of cobalt is removed from the electrolytic vat in a continuous manner, thereby preventing the accumulation of the oxid at the bottom of the electrodes which would 30 tend to short circuit the system. Furthermore, as a result of the directional flow of the electrolyte, the oxid of cobalt is prevented from adhering to the anode and finally causing a short circuit between the 35 anode and the adjacent cathode. This process may be carried out in any suitable electrolytic apparatus by arranging the streams of the electrolyte in such a manner that they cause a downwardly directed current across 40 the anode electrodes at the proper speed.

In the accompanying drawings is shown one form of apparatus which may be utilized to carry out the process.

In the drawings: Figure 1, is a center vertical section of an electrolytic vat taken in a plane parallel to the electrode plates; and Fig. 2 is a side elevation partly in section of the vat shown in Fig. 1 and at right angles to this figure.

45 In carrying out my improved process the terminal plates or electrodes are arranged parallel to each other in a suitable retaining vessel or vat with an inlet for a continuous supply of electrolytic solution directed between the members of each pair of electrodes. The electrolyte flows in a practically continuous stream from the inlets and passes between and in contact with the electrodes so that the entire surface of each electrode 50 or at least the anode electrode is subjected to the action of the continuously passing current. The velocity of the stream may be controlled in any desired manner and is always sufficient to retard if not to 55 prevent entirely the rising of the liberated

chlorin gas. Preferably, the direction of flow is substantially downward and transverse to the face of the electrodes and the best results are attained when the flow is vertically across the electrodes.

70 Preferably the outlet is located at a point below the bottom of the electrodes so that the flow of electrolyte will be in approximately the same path as the naturally falling precipitates. The precipitates of cobalt 75 oxid may be separated from the withdrawn solutions in any suitable manner, as by filtering or by depositing the same in suitable settling boxes, or the entire electrolyte, carrying the suspended oxids, may be returned to the electrolytic vat and the operation repeated.

80 In the particular apparatus shown in the accompanying drawings, the vat 4 may be of rectangular section provided with a hopper bottom 5 having an outlet 6 at its lowest point. Plate electrodes 7 are suspended in the upper portion of the vat by straps 8 depending from cross-bars 9 resting on the main bus bars 10. Supply pipes 11, communicating with the source of supply of the solution, are led along each side of the vat and have a plurality of discharge outlets 12 projecting down into the vat. The orifices of these outlets are pointed in a general downward direction toward the outlet 6. The electrolyte is drawn out through the outlet by any suitable means, such as a pump, at substantially the same rate as it is fed to the vat through the various supply 90 pipes and therefore there is at all times a generally downward current of electrolyte 95 serving to prevent the chlorin gas from rising through the solution and escaping. The speed of this current will of course depend 100 on the quantity of electrolyte supplied to a given size tank through the orifices, and drawn from the tank through the outlet. I have found that with a tank having a capacity of about 240 gallons, good results 110 may be obtained by feeding the solutions thereto and drawing the out-flowing stream therefrom at the rate of from 40 to 80 gallons per minute.

115 In the foregoing description of the process it is stated that a basic neutralizing agent, such as sodium carbonate, is added with the cobalt solution to the electrolytic vat and is present during the electrolysis. As the object of this agent is to neutralize 120 any free acid which might dissolve the cobalt oxids formed, it is obvious that the flow past the electrodes and the handling of the oxids may be carried on so rapidly that the small amounts of acid formed are prevented from acquiring a concentration which 125 might dissolve the cobalt oxids. Due to the activity with which sodium carbonate precipitates cobalt from its solution, it is preferable to add the neutralizing re-agent after 130

the solution has passed the electrodes and after the oxids have formed. In one successful working of the process the base is added to the flow after it has passed from 5 the electrolytic vat.

Having thus described my invention, I claim:

1. In the art of obtaining cobalt oxids from a solution containing a soluble cobalt 10 salt, the process which consists in subjecting the solution to an electrolytic action in the presence of a soluble chlorid, passing the solution in a downwardly directed current at a speed permitting the retention 15 of the chlorin gas liberated in the solution thereby to form a hypochlorite and permitting the hypochlorite so formed to react on the solution of cobalt in the presence of an agent capable of preventing the formation 20 of any free acid in the solution.

2. In the art of electrolytically extracting cobalt oxids from solutions containing a soluble chlorid and soluble cobalt salt, the process which consists in causing a current 25 of the electrolytic solution to pass across the anode electrode in a direction and at a velocity to retain in the solution any chlorin gas generated adjacent the electrode by the electrolytic treatment of the solution.

3. In the art of electrolytically extracting cobalt oxids from solutions containing a soluble cobalt salt, the process which consists in subjecting the solution to an electrolytic action in the presence of a coacting 35 chlorin-forming-agent and causing all of the free chlorin so formed to react chemically upon the solution.

4. In the art of electrolytically extracting cobalt oxids from solutions containing a 40 cobalt salt and a soluble chlorid, the process which consists in directing the solution downwardly past the anode electrode and in the presence of an agent, designed to neutralize any acid which may be formed adjacent the anode.

5. In the art of forming cobalt oxids from a solution containing cobalt and nickel salts, the process which consists in subjecting the solution to an electrolytic action in the presence 45 of a basic neutralizing agent and in the

presence of free chlorin gas retained in the solution.

6. In the art of extracting cobalt oxids from solutions containing a soluble cobalt salt, the process which consists in subjecting 55 the solution to an electrolytic action in the presence of chlorin and a neutralizing agent while causing the solution to pass the electrodes at a rate sufficiently rapid to remove any precipitates from the electrodes. 60

7. In the art of extracting cobalt oxids from solutions containing a soluble cobalt salt, the process which consists in subjecting 65 the solution to the action of a hypochlorite in the presence of an agent capable of preventing the formation of any solvent of the cobalt oxid formed.

8. The improvement in the art of forming cobalt oxids, which consists in subjecting a 70 solution containing a soluble cobalt salt, a soluble chlorid and a neutralizing agent to an electrolytic action, the neutralizing agent being added at a rate just sufficient to maintain a neutral or substantially neutral condition in the solution. 75

9. In the art of forming cobalt oxids from a solution of cobalt salts, the process which consists in subjecting the solution to the action of free chlorin in the presence of a 80 neutralizing agent.

10. In the art of extracting cobalt oxids from solutions containing cobalt salts, the process which consists in subjecting the solution to an electrolytic action in the presence of an agent which will react therewith to 85 form a free acid and automatically removing the acid incidentally formed at a rate which will prevent its accumulation and consequent concentration.

11. In the art of extracting cobalt oxids 90 from solutions containing cobalt salts, the process which consists in subjecting the solution to an electrolytic action and automatically removing the acid incidentally formed at a rate which will prevent its accumulation and consequent concentration. 95

Signed at New York, in the county of New York, and State of New York, this 17<sup>th</sup> day of August, A. D. 1915.

KENNETH S. GUITERMAN.